

# UNITED STATES PATENT OFFICE.

ROBERT ATHELSTAN MARR, OF NORFOLK, VIRGINIA, ASSIGNOR TO AMERICAN WOOD ENCYSTING CO., INCORPORATED, OF NORFOLK, VIRGINIA, A CORPORATION OF VIRGINIA.

## PROCESS OF TREATING WOOD FOR BUOYANT ARTICLES AND PRODUCT THEREOF.

1,121,645.

Specification of Letters Patent.

Patented Dec. 22, 1914.

No Drawing.

Application filed January 13, 1914. Serial No. 811,909.

To all whom it may concern:

Be it known that I, ROBERT ATHELSTAN MARR, citizen of the United States, residing at Ghent, Norfolk, in the State of Virginia, have invented certain new and useful Improvements in Processes of Treating Wood for Buoyant Articles and Products Thereof, of which the following is a specification.

The present invention relates to the treatment of woods of low specific gravity, to render them particularly suitable for use in making various buoyant articles, such as life preservers, fenders, floats, buoys and the like.

It is a well known fact that certain varieties of wood, particularly balsa and ceiba woods, are very light, that is they possess a very low specific gravity (about .25) and it has been proposed to use these woods in place of cork in life belts and similar devices, but it has been found that these woods are not entirely suited for the purposes mentioned, for the reasons, first, that they readily absorb and take up large quantities of water, which greatly decreases their buoyancy and secondly these varieties of wood are very susceptible to decay and insect attack, such as attacks by teredo and other wood destroying organisms. These objectionable properties render the wood in its natural condition, unsuited for use in life preservers and in substantially all buoyant articles, and accordingly most of the suggestions heretofore made for so employing these varieties of wood have not been entirely successful.

In my prior U. S. patents, dated April 16, 1912, Nos. 1,023,745 and 1,023,784, I have described two processes in which different kinds of wood can be impregnated by various materials including melted paraffin, which processes will prevent the absorption of water by the woods, and which will also prevent decay, and the ravages of various marine insects and other similar wood destroying agencies.

In my copending application Serial No. 747,169, filed Feb. 8, 1913, I have described a process of preserving wood, by the treatment of wood with a bath containing paraffin, naphthalene and diatomaceous earth, which process, I have now found to be particularly suitable for the application to the

varieties of wood above referred to, and I have also found that certain modifications 55 of this process are also capable of producing excellent results in the treatment of woods of these stated varieties and similar kinds of wood, suitable for use in the production of buoyant articles, as well as for 60 structural purposes.

In carrying out my present invention, wood in pieces of suitable size and shape for use in making the life preservers or other articles above referred to is subjected to the 65 action of a bath comprising paraffin, naphthalene and diatomaceous earth, to which bath a small amount of rosin and of Paris green may or may not be added depending upon whether or not the production of certain properties referred to later on is desired. This bath will preferably be maintained at a temperature somewhat above the boiling point of water, a temperature of 75 250° F. being suitable, during the action of 70 which bath, the moisture content of the wood is largely or entirely driven out, and more or less of the bath is absorbed by the wood. The temperature of the bath may be lowered more or less, depending upon the 80 amount of impregnation or encysting of the wood which is desired. For the production of blocks of wood for use in life preservers, it is ordinarily not necessary or desirable to give a heavy impregnation, for 85 the reason that it is desirable to produce a finished product, having as low a specific gravity as possible, in order to have a high buoyant effect. In order to produce the low impregnation, I preferably do not allow 90 the temperature of the bath to fall more than a few degrees, say from 250° F. at the beginning of the operation, down to 180 or 200° F., at which point the wood is preferably removed from the bath, and allowed 95 to further cool to ordinary temperature.

Instead of allowing the temperature of the entire bath to fall, after the wooden articles have been immersed in the hot bath for a short time, at a temperature of 250° F. 100 (more or less) I may remove said articles from the bath, and immerse the two ends of the same (first one end and then the other) in a bath of similar composition, or another bath, maintained at a temperature 105 of 180° F. (more or less). The second bath

- obviously may consist of the same materials, and in the same proportions, as I used in the first bath, the temperature of said bath being lower, or if desired, the second bath 5 may consist of the same materials, and in different proportions from the first bath, or if desired, the second bath may consist of different materials from those employed in the first bath: Any liquid, or material which 10 is liquid at the temperature desired for the second bath, say 180° F., which is not injurious to the wood, or to the ingredients of the first bath, may be employed for this second bath.
- 15 The time of immersion and cooling may vary more or less depending on the size of the wooden pieces, the amount of impregnation desired, moisture content of the wood, and other factors, but I have found that for 20 blocks of balsa wood of two inches square, and four inches long, a hot bath for five minutes and then cooling to 180° F., during two minutes, has been found to give excellent results.
- 25 The impregnation of the surface portions of the wood is in this manner made quite complete, while the interior portions of the wood are not saturated with the impregnating material; but a small amount of the material will be carried, by means of the large 30 ducts existing in these varieties of wood, practically throughout the body of the material, whereby the paraffin, naphthalene and diatomaceous earth, are caused to be 35 thoroughly disseminated in very small amounts, throughout the entire body of the wood, while the small air spaces throughout the body of the wood are not filled with the impregnating material.
- 40 In this way I can produce blocks having very low specific gravities which will be thoroughly and completely waterproofed, and preserved against rot, and attack of marine insects and similar wood-destroying 45 agencies.
- As a modified mode of procedure, I can incase the blocks of wood, in the duck, canvas or other fabric forming the body of the life belt or similar structure, and then treat 50 the finished article by the process of impregnation, which not only preserves the wood, but also preserves the fabric against the destructive agencies such as dry rot and the like, and makes it waterproof.
- 55 In making certain other kinds of buoyant articles, it is not desired to produce such a high degree of buoyancy, instances of this being buoys for anchoring boats and the like, and in the treatment of articles of this 60 character, I find that a heavy impregnation of the article with the preservative specified is a material advantage, since these articles are likely to be deeply chipped by the action of boats striking the same, and a complete 65 impregnation or substantial saturation of

the woods in question is particularly advantageous, in order to insure the article against decay or insect attack, at those points where the article has received injury.

In producing the heavy impregnation, in 70 such cases as above referred to, I preferably introduce the wood, in a rather moist condition, into a bath of the specified materials, at a somewhat higher temperature, say 250 to 275° F., 260 being preferred, then allow 75 the temperature to drop slowly, while the wood is immersed in the liquid, to a temperature down to near the solidifying point of the treating bath.

For treating wood for the construction of 80 boats, particularly life boats and the like, I subject the material to a heavy impregnation, which gives considerably more strength to the material, than would be produced by a light impregnation.

In carrying out the impregnation process in all the modifications the material is immersed and held under the surface of the bath. I desire to call attention to the fact that the wood when so treated, may be 90 coated, if so desired, over all or a part of its surface with paint, either for ornamentation, or marking purposes. In using ordinary paint, it is preferable to first apply a 95 coat of shellac.

If desired I may add to the impregnating bath any suitable oil-soluble dye, which will be carried into the wood, wherever the preservative is carried.

The bath used in impregnating the material may consist of the materials in the following proportions by weight, although the invention is not limited thereto, and the proportions may be materially altered without departing from the spirit of the invention; 100 paraffin 100 parts, naphthalene 3 to 7 parts, diatomaceous earth 2 to 7 parts, (to which may be added if desired, rosin 2 to 5 parts, or Paris green 1 part, or both.)

The naphthalene employed in this process acts as a conveying agent, for carrying the paraffin, together with the diatomaceous earth suspended therein, into the pores and ducts of the wood. The naphthalene also 115 exercises a preserving action upon the wood.

The use of Paris green in this connection is materially different from the diatomaceous earth, since it is not carried into the interstices of the wood, to any great extent, but remains as a surface coating on the surface of the wood.

The use of rosin is, as above stated, somewhat optional. This material hardens the wood to a considerable extent, also makes the wood tougher, and gives a somewhat adhesive condition to the surface of the wood, thereby making the treated material more easy to cling to.

The wood for ring buoys may be made in the form of rings, which may be "built up" 130

(composed of three or more layers, united by a suitable waterproof glue) if desired, and these may be covered by duck or the like, before impregnation, if desired. Also 5 I may treat the wood in the form of large pieces, logs or the like, and afterward, if small pieces are needed I may cut this to produce pieces of the proper size for the particular use, if so desired. This method 10 is not to be generally recommended, in the case of material having a very light impregnation, since it is desirable to have a rather heavy superficial impregnation over the surface portions of the article. For 15 light impregnation, I may use wood in its air dry condition, to advantage, while for heavy impregnation I preferably use wood which is more or less saturated with water, or sap. Green wood, directly after being 20 cut is suitable. It is my opinion, that the dissemination of the preservative throughout the body of the wood, is aided by osmosis.

The treatment of wood with a mixture including 25 paraffin, rosin and diatomaceous earth, with or without Paris green, and a dye soluble in the bath, is claimed in my copending application Serial No. 811,910, filed Jan. 13, 1914. The treatment of fabrics 30 and other textile materials, by the methods herein disclosed is described and claimed in my copending applications Nos. 811,911 and 811,912, both filed Jan. 13, 1914.

What I claim is:—

- 35 1. A process of treating woods of low specific gravities in their natural condition, which comprises impregnating said woods with a hydrocarbon material containing a finely divided solid material.
- 40 2. A process of treating woods of low specific gravities, which comprises impregnating said woods in their natural condition, with hydrocarbon material containing a finely divided solid material.
- 45 3. A process of treating woods of low specific gravity, which comprises immersing said woods in a bath comprising paraffin, diatomaceous earth and a conveying agent, while said wood contains some moisture.
- 50 4. A process of treating moist woods of low specific gravities, said process comprising immersing the wood of the class specified, in a bath comprising paraffin, naphthalene and diatomaceous earth.
- 55 5. A process of treating wood of low specific gravity said process comprising the steps of placing said wood in a permeable envelop, and thereafter subjecting the same to a heated bath of paraffin, diatomaceous earth and a conveying agent.
- 60 6. A process of treating wood of low specific gravity, which comprises immersing the same in a bath containing paraffin, naphthalene and diatomaceous earth, at a temperature materially above the boiling

point of water, then treating the same with a bath at a temperature lower than that employed in said first treatment.

7. A process of treating balsa and ceiba wood, which comprises treating the same 70 with a bath containing diatomaceous earth, a vehicle insoluble in water and a material capable of increasing the rate of penetration of said vehicle.

8. A process of treating balsa, ceiba and 75 similar varieties of wood which comprises treating the same with a bath comprising paraffin, naphthalene and diatomaceous earth, at a high temperature, then with a bath composed of materials not injurious to the 80 wood, or to the ingredients of said first bath, said second bath being at a lower temperature, until the desired impregnation is secured.

9. A process of treating balsa, ceiba, and 85 similar varieties of wood which comprises treating the same with a bath comprising paraffin, naphthalene, rosin and diatomaceous earth, at a high temperature, then with a bath capable of increasing the amount of 90 absorption of said first bath, said second bath being at a lower temperature, until the desired impregnation is secured.

10. A process of treating balsa, ceiba, and 95 similar varieties of wood, which comprises treating the same with a bath comprising paraffin, naphthalene, rosin, Paris green, and diatomaceous earth, at a high temperature, then with a bath containing at least some of the ingredients of said first bath, said second 100 bath being at a lower temperature, until the desired impregnation is secured.

11. A process of treating balsa, ceiba, and 105 similar varieties of wood which comprises treating the same while incased in a fabric cover with a bath comprising paraffin, naphthalene and diatomaceous earth, at a high temperature, then with a bath containing paraffin at a lower temperature, until 110 the desired impregnation is secured.

12. A process of treating balsa, ceiba, and other similar varieties of wood, which comprises subjecting the same to the action of a bath containing paraffin, naphthalene, diatomaceous earth and rosin.

13. A process of treating wood of those varieties having a relatively low specific gravity, which comprises immersing the same in a bath comprising paraffin, naphthalene, rosin, Paris green, and diatomaceous 120 earth.

14. An article of manufacture comprising a wood of relatively low specific gravity impregnated with a preservative including diatomaceous earth, a vehicle comprising 125 paraffin and a somewhat volatile, aromatic hydrocarbon.

15. An article of manufacture comprising a wood of relatively low specific gravity, 130 impregnated with a preservative including

- diatomaceous earth, and a vehicle comprising paraffin and naphthalene.
16. An article of manufacture comprising a wood of relatively low specific gravity, 5 impregnated with a preservative including diatomaceous earth, and a vehicle comprising paraffin, naphthalene, and rosin.
17. An article of manufacture comprising a wood of relatively low specific gravity, 10 impregnated with a preservative including diatomaceous earth, and a vehicle comprising paraffin, said wood having a casing of fabric impregnated with a similar preservative.
18. An article of manufacture comprising a balsa wood, impregnated with a preservative including diatomaceous earth, and a vehicle comprising paraffin.
19. An article of manufacture comprising wood of relatively low specific gravity, 20 impregnated with a preservative material including an insoluble finely divided solid material, having a hardness greater than that of the material of which the biting parts of marine wood-destroying worms is composed, 25 and an insoluble hydrocarbon carrier which
- melts at a temperature below the boiling point of water, and which is solid at ordinary temperatures, and a material capable of increasing the rate of penetration of said preservative material. 30
20. An article of manufacture comprising wood of relatively low specific gravity, impregnated with a preservative material including an insoluble finely divided solid material, having a hardness greater than that 35 of the material of which the biting parts of marine wood-destroying worms is composed, and an insoluble hydrocarbon carrier which melts at a temperature below the boiling point of water, and which is solid at ordinary temperatures, said wood being coated with a material including an insoluble poisonous compound. 40

In testimony whereof I have affixed my signature in presence of two witnesses.

ROBERT ATHELSTAN MARR.

Witnesses:

JANEY HOPE MARR,  
A. B. FOSTER.